

J. E. YORK.

PROCESS OF ROLLING INGOTS.

APPLICATION FILED JULY 14, 1906.

1,078,119.

Patented Nov. 11, 1913.

2 SHEETS—SHEET 1.



FIG. 1.



FIG. 2.

FIG. 3.



FIG. 4.



FIG. 5.



INVENTOR :

James E. York

By Attorneys,

Julian O. Draper & Meina

WITNESSES:

Fred White

Rene' Muine

1,078,119.

J. E. YORK.  
PROCESS OF ROLLING INGOTS.  
APPLICATION FILED JULY 14, 1906.

Patented Nov. 11, 1913.

2 SHEETS—SHEET 2.

FIG. 6.



FIG. 7.



FIG. 8.



FIG. 9.



WITNESSES:

Red White

Rene Bruine

INVENTOR :

James E. York

By Attorneys,

Arthur G. Draper & Maria

# UNITED STATES PATENT OFFICE.

JAMES E. YORK, OF NEW YORK, N. Y.

## PROCESS OF ROLLING INGOTS.

1,078,119.

Specification of Letters Patent.

Patented Nov. 11, 1913.

Application filed July 14, 1906. Serial No. 326,211.

*To all whom it may concern:*

Be it known that I, JAMES E. YORK, a citizen of the United States, residing in the borough of Brooklyn, county of Kings, city and State of New York, have invented certain new and useful Improvements in the Process of Rolling Ingots, of which the following is a specification.

This invention relates to the rolling of iron or steel shapes from the ingot to produce a product the body of which is either in the original condition left by casting the ingot, or is reduced by longitudinal rolling (so that it has a longitudinal grain), such body having a lateral flange or flanges produced by transverse rolling, so that the grain thereof is transverse.

The invention may be applied to a cast steel ingot, or this may be reduced by longitudinal rolling in the ordinary manner to a bloom or other elongated steel shape. Or any suitable form of wrought iron may be used; for example, muck bars rolled into a bloom of proper sectional area which may or may not be further reduced by longitudinal rolling.

According to the present invention the ingot, bloom or other elongated shape of iron or steel, is placed on a support and rolled transversely to cause the portion thus rolled to extend beyond the body of the steel or iron shape to form a lateral flange. The support may be any suitable bed or table adapted to support the ingot or other steel shape, not only underneath but also laterally to the necessary extent, while it is subjected to the action of a roll over it, extending parallel or nearly so with the steel shape and moving relatively to the support, so that the rolling action is transverse to the longitudinal dimension of the steel shape. For this purpose either the roll may move over a stationary support, or preferably the support is formed as a movable bed which travels beneath the stationary roll. The support or bed is formed with transverse grooves or depressions each suitably shaped to receive and substantially conform to the under portion of the steel shape, which however is only partially embedded in the depression, its upper portion projecting above the support, so that the rolling operation takes effect solely or chiefly upon this protruding portion, whereby it is spread laterally to form a flange or flanges. After the upper side of the steel

shape has thus been laterally flanged, it may be inverted in a suitably shaped recess and its under (now its upper) side may be similarly flanged. The laterally rolled or flanged shape may then be subjected to further longitudinal rolling, whereby to reduce its section to the desired finished contour. Or the flanged shape may be finished by forging, bending or other metal-working process.

The present invention enables a great variety of beams, girders, columns, and other forms of structural steel to be rolled, having flanges of far greater width than could possibly be produced by longitudinal rolling, and renders feasible the production of various sections that it would be impossible or impracticable to produce by longitudinal rolling alone.

Referring to the accompanying drawings,—Figure 1 is a vertical section in the plane of the travel of the bed, showing a rolling mill adapted to the practice of the present invention, and showing the steel in successive stages of the process of rolling; Fig. 2 is a fragmentary section in the same plane showing the bed adapted to further stages in the process of rolling; Figs. 3, 4 and 5 are perspective views of the ingot or bloom before rolling, and of the flanged products made therefrom; Fig. 6 is an elevation of longitudinal rolls for the subsequent reduction of a transversely flanged shape such as is shown in Fig. 5; Fig. 7 is a vertical section showing a fragment of Fig. 1 or Fig. 2 and illustrating a further modification of the bed; Fig. 8 is an elevation of a longitudinal rolling mill adapted for the subsequent reduction of a transversely flanged shape such as is shown in Fig. 7; Fig. 9 is an elevation of another rolling mill for the subsequent longitudinal rolling to a more complicated shape.

Referring to Fig. 1, let A designate the support or bed and B the roll. The bed A may be made of a lower part or base plate C and an upper or grooved plate D, which latter may be made in sections to advantage, three of such sections being shown at D'. The bed is preferably made to travel beneath the roll B, for which purpose it may advantageously be supported on rollers E E beneath. The roll B may be supported in any suitable side frames or housings F, and to reinforce its middle portion against deflecting strains it may have an auxiliary

roll G mounted above it. The bearings for the roll B (and roll G if used) should be vertically adjustable as by means of any known or usual adjusting screws H, or by any other suitable means.

Fig. 3 shows a metal shape *a* upon which the transverse rolling operation is to be performed. This may be the cast ingot, or a bloom or other shape reduced from an ingot, or from muck bars or the like, by any suitable hammering, rolling or other reducing operation. Whether the transverse rolling of the present invention is performed upon a cast ingot, or rolled bloom, or other shape, will depend upon the purpose to be fulfilled. The original steel shape *a* is placed in a groove or depression L formed in the top of the support or bed A, this groove being preferably as close a fit as practicable with the sides of the steel shape, and of a depth such as to leave a portion thereof projecting above the top of the bed as shown. By use of a sectional bed the shape may be clamped tightly in the groove by means of any clamping device, such as a screw M. The bed is then moved under the roll B, which is adjusted downward so as to bear upon and laterally displace the upper or protruding portion of the steel shape *a*. After each pass beneath the roll, the roll is adjusted lower so that by a succession of passes the protruding portion of the steel shape is displaced laterally to form a flange which is spread over the upper surface of the bed. At *b* in Fig. 1 is shown the steel shape after being rolled transversely to form a flange *c* projecting to both sides. Thus is formed the product shown in Fig. 4. This product is characterized by its body or web portion *d* having its grain unchanged, being either the crystalline structure left in casting, or the longitudinal grain resulting from an initial rolling; and by its flange *c* having a transverse grain produced by the rolling action of the roll B. This grain is shown by the surface tinting in Fig. 4.

If it is desired to make the flange *c* tapered, the top of the bed may be made with the desired bevel as shown at N Fig. 1, so that the flanged shape is given the desired taper beneath its flange as shown in sectional shape *d* Fig. 1. In case it is not desired to limit the width or thickness of the flange *c*, this flange is formed by rolling directly upon the top of the bed as shown at *b* in Fig. 1. If, however, it is desired to limit the width and thickness of this flange, an auxiliary depression L' is provided into which to spread the flange by lateral rolling, as shown in the sectional shape *e* in Fig. 1. The bottoms or edges of these auxiliary depressions may have any special conformation which it is desired to impart to the flanges, whereby they may be ribbed, beaded, embossed, or otherwise varied.

If it is desired to form a flange *c* on both sides of the original shape whereby to produce a product such as that shown in Fig. 5, this is performed by turning over the shape *b* *d* or *e* (Fig. 1), placing it inverted in a suitably shaped recess L<sup>2</sup> in the same or another bed (see bed A' Fig. 2), and then rolling what was formerly its lower but is now its upper side to form the additional flange, the latter being shown at *f* in Figs. 2 and 5. For convenience in entering the shape into the recess L<sup>2</sup>, this is best made with its lower enlargement deeper than the width of the flange *c*, the excess being filled by a wedge or filling piece O.

The modified or flanged ingot or bloom produced by this invention, examples of which are shown in Figs. 4 and 5, may have its body portion and flange or flanges variously proportioned according to its intended purpose. Such modified ingot or bloom may be subjected to any desired or appropriate subsequent manipulations according to the article that it is desired to produce. For example, it may be subjected to subsequent longitudinal rolling between such rolls as those shown at P' Q in Fig. 6, these particular rolls being adapted to act upon the steel shape shown in Fig. 5 (or that shown at *g* or *h* in Fig. 2) for reducing its section to the final section desired, thereby proportionally elongating it. For this purpose the rolls have passes R, S, T, U, adapted to successively reduce the section.

The improved process is adaptable to the production of sections having excessively wide or deep flanges, such for example as that shown at *i* in Fig. 7. For such sections it is only necessary that the bed be constructed with its sections of proper shape to form intervening grooves of the requisite contour. The section *i* may be reduced originally from the ingot *a* Fig. 1, or from an already flanged shape such as those shown at *g* or *h* in Fig. 2.

In the case of sections having flanges too wide to be properly reduced by longitudinal rolling in a closed pass between rolls such as are shown in Fig. 6, the longitudinal rolling is best performed by a four-roll mill such as shown in Fig. 8, having opposite rolls P' P' entering between the flanges against the web portion, and lateral rolls V V engaging the outer faces of the flanges and reducing them against the side faces or formers of the rolls P' P'. The latter may be horizontal rolls, and the rolls V V may be vertical rolls, or vice versa. The rolls shown in Fig. 8 are adapted for reducing the section *i* shown in Fig. 7. The respective rolls may have projections or formers adapted to indent, bend, flange, or otherwise change the shape of the web portion or flanges as desired. An example of this is shown in Fig. 9, where the rolls W W

70

75

80

85

90

95

100

105

110

115

120

125

130

serve for bending out the flanges against the rolls Y Y, which latter have angular formers adapted to shape the flanges, and also to turn their outer edges against the 5 sides of the rolls W to form edge flanges thereon. The flanged section k shown in Fig. 9 is useful as an integral column, and is a section which it would be extremely difficult or impossible to produce by ordinary longitudinal rolling methods.

The present invention is related to that set forth in my application No. 177,989 filed October 21, 1903, which however was directed more particularly to the re-rolling of 15 old or worn rails, beams, girders, etc., for producing various laterally flanged shapes. In that application the process is performed normally upon steel already reduced by longitudinal rolling, and after the transverse 20 rolling process has been completed normally no further longitudinal rolling is performed. The process of the present invention starts with steel or iron in substantially a raw condition, that is to say, in 25 the form either of the original ingot, or of a bloom or billet, or other crude shape produced by an insignificant amount of longitudinal rolling, the major portion of the redistribution required to produce the desired 30 shape being performed by transverse rolling according to the process of the present invention, after which any desired further reduction, elongation or bending to produce the ultimate section may be performed by 35 longitudinal rolling, or by bending, forging or other means.

Where the process is applied to a cast steel ingot, it has the additional advantageous effect of compacting the surface of the ingot 40 so as to close the blow holes which ordinarily lie near the surface, and to close any central voids in the ingot such as sometimes exist by reason of the failure to crop off the entire pipe. Occasionally, although the end

of the ingot, after cropping, looks solid, 45 there is some slight piping below this end, and the present process compacts the ingot so as to close any such pipes.

Though I have described with great particularity of detail certain processes and 50 products embodying this invention, yet it is not to be understood that the invention is limited necessarily thereto, since various modifications may be made by those skilled in the art, without departing from the in- 55 vention.

What I claim is:—

1. The process of treating an ingot or bloom, which consists in holding it in a support with its sides engaged by said support 60 and in a position in which its edge extends above said support and subjecting the exposed edge of it to a succession of transverse rolling operations by a roll supported above and out of contact with said support 65 sufficient to roll it out into a flange extending laterally beyond the body and resting on said support.

2. The process of treating an ingot or bloom, which consists in subjecting it to 70 transverse rolling to upset the metal and form a flange and then reducing the flanged shape thus formed by longitudinal rolling.

3. The process of treating a cast ingot which consists in rolling an edge of it transversely to points beyond the body of the ingot 75 so as to form a flange and under sufficient pressure to upset the metal and compact the flange so as to form a lateral grain therein.

In witness whereof, I have hereunto signed my name in the presence of two subscribing witnesses.

JAMES E. YORK.

Witnesses:

ARTHUR C. FRASER,  
FRED WHITE.

Copies of this patent may be obtained for five cents each, by addressing the "Commissioner of Patents, Washington, D. C."